

# UNITED STATES PATENT OFFICE.

PEDER FARUP, OF CHRISTIANIA, NORWAY, ASSIGNOR TO TITAN CO. A/S. OF NORWAY,  
OF CHRISTIANIA, NORWAY.

## PROCESS OF PRODUCING TITANIUM COMPOUNDS.

1,343,441.

Specification of Letters Patent. Patented June 15, 1920.

No Drawing. Application filed February 27, 1918, Serial No. 219,407. Renewed April 4, 1919. Serial No. 287,631.

To all whom it may concern:

Be it known that I, PEDER FARUP, a subject of Norway, and a resident of Christiania, Kingdom of Norway, have invented 5 certain new and useful Improvements in Processes of Producing Titanium Compounds, of which the following is a specification.

This invention relates to the manufacture 10 of titanium compounds, which are suitable for the production of pigments and for other purposes.

The object of the invention is a method 15 whereby such compounds can be produced from titaniferous iron ores with great economy, the method giving as a by-product nitrogen compounds suitable for use as fertilizers.

As a raw material for my process I can 20 use any titaniferous material, but I prefer to use materials which occur in nature, especially ilmenite or similar titaniferous iron ores, as these are the titanium materials most readily available.

25 Broadly speaking the invention is carried out by heating such a titaniferous material containing iron together with a reducing agent in an atmosphere of nitrogen until a reaction takes place whereby a titanium nitrogen compound, for example  $TiN_3$ , is formed, and the iron present is reduced to the metallic state. If the reducing agent employed is carbon, there will be formed in addition to titanium nitrid, also titanium 30 cyanonitrids. The iron is then removed from the titanium nitrogen compound either by means of magnetic separation or by means of an acid which will dissolve the iron but not the titanium compounds. I 35 have found that in this way the principal part of the iron compounds may be easily separated from the titanium compounds and that the latter are brought into a condition which is suitable for further treatment. I 40 have found that concentrated sulfuric acid will easily react with the above mentioned titanium nitrogen compounds even when employed in a comparatively small quantity. The decomposition is quickly 45 started by the application of initial heat; but as the reaction is exothermic, no further heating is necessary after the reaction is once started. The reaction will proceed with considerable speed and violence until a com-

plete decomposition has taken place. After 55 the reaction has been completed the resulting product forms a solid mass if the right amount of sulfuric acid has been employed. I have found that this solid mass contains practically all the nitrogen of the titanium 60 nitrogen compound in the form of ammonium sulfate and also titanium sulfate and small amounts of iron in the form of ferrous sulfate. These sulfates are soluble in water and on lixiviation a solution containing all these sulfates will result. From 65 this solution the titanium may be precipitated in well known manner. As the iron in the solution is present in the divalent state and the titanium to a great extent in 70 the trivalent state it is possible to effect a practically complete separation of titanium 75 compounds from iron compounds by precipitation by means of heating when care is taken that sufficient trivalent titanium is 80 present to prevent the oxidation of divalent iron to trivalent iron. In this connection reference may be had to Norwegian Patent No. 28,088, which is embodied in U. S. application Sr. No. 196,316, filed October 12, 1917. The resulting precipitate, consisting 85 principally of titanium hydrates and containing an undesired acid substance and traces only of iron, is well adapted to further treatments whereby the said acid substance is eliminated and whereby the product resulting therefrom is by calcination converted wholly or partly into crystalline titanium dioxid which possesses excellent 90 qualities as a pigment.

In this connection reference may be had to Norwegian Patent No. 27,604 which is embodied in United States application Sr. Nos. 196,978 and 196,979, both filed October 12, 1917, and Norwegian Patent No. 28,216 95 which is embodied in United States application Sr. No. 196,327, filed October 12, 1917.

The solution from which the titanium hydrates were precipitated may be further treated to recover the ammonium sulfate, 100 iron sulfate and free sulfuric acid remaining in the solution.

By utilizing the property of titanium to combine with gaseous nitrogen in considerable quantities, I have found a method for 105 producing titanium compounds which is applicable not only to the comparatively expensive pure titanium compounds but also to the

- titaniferous iron ores. At the same time that nitrogen is fixed by the titanium of said ores the iron also contained therein is changed to a condition which facilitates its separation from the titanium compounds. Further I have found that by this reduction process the titanium compounds present which serve to fix gaseous nitrogen are transformed to a condition in which they are 10 easily attacked by acids or other reagents, and are consequently in a form suitable for refining and manufacture of pure titanium compounds such as are used as pigments in paints and for other purposes.
- 15 The details of the various steps in my process may vary according to the raw material used and the final products desired. In the following specific illustration I will make use of ilmenite as a raw material and 20 carry out my process so as to obtain on one hand a titanium compound suitable for use as pigment, and on the other hand ammonium sulfate suitable for use as a fertilizer. The iron present in the ilmenite is transformed to ferrous sulfate. To carry out my process I proceed as follows: Ilmenite containing approximately 45%  $TiO_2$  and 40% Fe. is finely pulverized and mixed with pulverized carbon in a sufficient amount to reduce the iron oxids present to metallic iron and also the titanium oxid to titanium. I generally use an excess of carbon as losses may occur during the heating process and also titanium-cyanonitrid may be formed. 30 The mixture is brought into a furnace, preferably an electric furnace, which is supplied with nitrogen during the whole treatment, and heat applied until the iron is reduced to the metallic state and a titanium nitrogen compound is formed. Temperatures from 40 1200° to 1400° C. have given good results.
- The application of heat is continued until the ilmenite is practically completely decomposed. This point can be determined by 45 examining a sample from the furnace. The material is then crushed to the fineness of coarse sand.
- This powder is subjected to lixiviation with dilute acid, preferably sulfuric acid, 50 and the lixiviation is conveniently carried out according to the counter current principle. The acid will dissolve out the iron but not the titanium nitrogen compound, and care is taken that sufficient acid is used to dissolve 55 all iron present. In this example I will for convenience only refer to sulfuric acid although it is understood that other acids such as hydrochloric and nitric can be used.
- From the lixiviation there results a solution 60 containing ferrous sulfate and a residue consisting principally of titanium nitrogen compounds together with silica and other impurities originally contained in the ilmenite. After being dried this residue is 65 in a suitable condition for further treatment

to recover therefrom the titanium and the nitrogen in the form of useful products. It is known from literature that titanium-cyanonitrids on heating in the presence of steam form  $NH_3$ , HCN and H, the titanium 70 being transformed to  $TiO_2$ . I can make use of these reactions in my process if it is desired to produce HCN, but in this specific illustration of my process I will produce ammonium sulfate from the nitrogen fixed by 75 titanium, as this can be accomplished by a very simple operation.

I mix the dried residue thoroughly with concentrated sulfuric acid in approximately the proportion two parts by weight of 90% 80 sulfuric acid to one part by weight of residue and place the mixture in a cast-iron vessel. The mixture is now heated by means of steam or hot air until reaction takes place. The heating is then discontinued and the reaction 85 proceeds throughout the whole mass. The reaction product is a solid mass, of grey color, consisting principally of titanium sulfate and ammonium sulfate with small amounts of ferrous sulfate. I have found 90 that when proceeding as described practically no nitrogen is lost.

The mass thus obtained may be subjected to various treatments for the manufacture of pure titanium compounds and ammonium 95 sulfate. I can heat the mass to above 400° C. whereby the sulfates of ammonia and titanium are decomposed. After lixiviation of the resultant mass with water or dilute acid, whereby the ferrous sulfate present 100 will dissolve, practically pure  $TiO_2$ , will remain as a residue. I prefer, however, to lixiviate the mass obtained by the treatment with sulfuric acid directly with water according to the counter current principle. 105

I then use about four parts by weight of water to one part by weight of solid mass. There results a concentrated solution of titanium sulfate, ammonium sulfate and small amounts of ferrous sulfate. The residue 110 consisting principally of silica from the original ore is then removed from the solution.

The solution is heated to boiling whereby titanium is precipitated in the form of a 115 hydrate containing a small amount of sulfuric acid. This is separated from the solution by means of filtering, washed, and is then in itself a valuable product. I prefer, however, to produce a pigment from this 120 product and to this end I treat it according to Norwegian Patent No. 27,604 with barium chlorid or similar compounds whereby the undesired acid substance containing the  $SO_4$  radical which comes down on precipitation 125 is neutralized. On calcination according to Norwegian Patent No. 28,216 I obtain a product consisting principally of titanium oxid partly or wholly in the crystalline form and also containing about 20% of barium 130

sulfate. As set forth in the said Norwegian patent a product consisting principally of  $TiO_2$  in the crystalline form and with the structure therein described is very well 5 adapted for use as a pigment. This pigment, however, I do not claim as my invention but only my method of producing it.

The solution from which the titanium hydrate has been precipitated contains ammonium sulfate, small amounts of iron sulfate and free sulfuric acid liberated by the precipitation of titanium hydrate. The ammonium may be recovered therefrom by means of distillation after an excess of a 15 base such as  $Ca(OH)_2$ , has been added to the solution. But as the solution contains a considerable amount of acid I prefer to evaporate the solution until ammonium sulfate crystallizes out. This is separated from 20 the solution and is then in a form suitable for use as a fertilizer. The iron contained therein will do no harm if the product is used as a fertilizer. If an absolutely pure ammonium sulfate is desired the product 25 above described may be refined according to known methods, such as a repeated crystallization.

The sulfuric acid which remains after the crystallization of ammonium sulfate I use 30 for the lixiviation of iron as described in the first part of my process.

What I claim as new and desire to secure by Letters Patent of the United States is:

1. The process of preparing titanium compounds from titaniferous material containing iron, which comprises heating a titaniferous material containing iron together with a reducing agent in an atmosphere of nitrogen until a titanium nitrogen compound is 35 formed and the iron present is reduced to the metallic state, dissolving said metallic iron in acid, and separating the solution from the residue containing the titanium nitrogen compound.

45 2. The process of preparing titanium compounds from titaniferous material containing iron, which comprises heating a titaniferous material containing iron together with carbon in an atmosphere of nitrogen until a titanium nitrogen compound is formed and the iron present is reduced to the metallic state, dissolving said metallic iron in acid, and separating the solution from the residue containing the titanium nitrogen compound.

55 3. The process of preparing titanium compounds from titaniferous material containing iron, which comprises heating a titaniferous material containing iron together with carbon in an atmosphere of nitrogen until a titanium-nitrogen compound and also another titanium-nitrogen compound containing carbon are formed and the iron present is reduced to the metallic state, dissolving said metallic iron in acid, and separating the solution from the residue containing the titanium-nitrogen compound, heating said residue together with sulfuric acid to form titanium 60

taining the titanium nitrogen compound and also the titanium nitrogen compound containing carbon.

4. The process of preparing titanium compounds from titaniferous materials containing iron, which comprises heating a titaniferous material containing iron together with carbon in an atmosphere of nitrogen until a titanium nitrogen compound is formed and the iron present is reduced to 70 the metallic state, dissolving said metallic iron in acid and separating the solution from the residue containing the titanium nitrogen compound, heating said residue together with sulfuric acid to form titanium sulfate and ammonium sulfate, and separating these sulfates.

5. The process of preparing titanium compounds from titaniferous materials containing iron, which comprises heating a titaniferous material containing iron together with carbon in an atmosphere of nitrogen until a titanium nitrogen compound is formed and the iron present is reduced to the metallic state, dissolving 75 said metallic iron in acid and separating the solution from the residue containing the titanium nitrogen compound, heating said residue together with sulfuric acid to form titanium sulfate and ammonium sulfate, dissolving 80 said sulfates in water, heating the solution thus formed until a titanium hydrate is precipitated, and separating the precipitate from the solution.

6. The process of preparing titanium compounds from titaniferous material containing iron, which comprises heating a titaniferous material containing iron together with carbon in an atmosphere of nitrogen until a titanium nitrogen compound is formed and the iron present is reduced to the metallic state, dissolving said metallic iron in acid and separating the solution from the residue containing the titanium nitrogen compound, heating said residue together with sulfuric acid to form titanium sulfate and ammonium sulfate, dissolving 90 said sulfates in water, heating the solution thus formed until a titanium hydrate is precipitated, separating the precipitate from the solution, and crystallizing 95 out the ammonium sulfate from the solution.

7. The process of preparing titanium compounds from titaniferous material containing iron, which comprises heating a titaniferous material containing iron together with carbon in an atmosphere of nitrogen until a titanium nitrogen compound is formed and the iron present is reduced to 100 the metallic state, dissolving said metallic iron in acid and separating the solution from the residue containing the titanium nitrogen compound, heating said residue together with sulfuric acid to form titanium sulfate and ammonium sulfate, dissolving 105 said sulfates in water, heating the solution thus formed until a titanium hydrate is precipitated, separating the precipitate from the solution, and crystallizing 110 out the ammonium sulfate from the solution.

115 8. The process of preparing titanium compounds from titaniferous material containing iron, which comprises heating a titaniferous material containing iron together with carbon in an atmosphere of nitrogen until a titanium nitrogen compound is formed and the iron present is reduced to 120 the metallic state, dissolving said metallic iron in acid and separating the solution from the residue containing the titanium nitrogen compound, heating said residue together with sulfuric acid to form titanium 125

130

- sulfate and ammonium sulfate, dissolving said sulfate in water, heating the solution thus formed until a titanium hydrate containing a small amount of the  $\text{SO}_4$  radical 5 is precipitated, separating the precipitate from the solution, washing the precipitate and treating it with a barium compound to form barium sulfate with the  $\text{SO}_4$  radical present.
- 10 8. The process of preparing titanium compounds from titaniferous materials containing iron, which comprises heating a titaniferous material containing iron together with carbon in an atmosphere of nitrogen until a titanium nitrogen compound 15 is formed and the iron present is reduced to the metallic state, dissolving said metallic iron in acid and separating the solution from the residue containing the titanium 20 nitrogen compound, heating said residue together with sulfuric acid to form titanium sulfate and ammonium sulfate, dissolving said sulfates in water, heating the solution thus formed until a titanium hydrate containing a small amount of  $\text{SO}_4$  radical 25 is precipitated, separating the precipitate from the solution, washing the precipitate and treating it with a barium compound to form barium sulfate with the  $\text{SO}_4$  radical present, and calcining the resulting product to form  $\text{TiO}_2$  and barium sulfate.
9. The process of preparing titanium compounds from titaniferous material containing iron, which comprises heating a titaniferous material containing iron together with carbon in an atmosphere of nitrogen until a titanium nitrogen compound 35 is formed and the iron present is reduced to the metallic state, dissolving said metallic iron in acid and separating the solution from the residue containing the titanium nitrogen compound, heating said residue together with sulfuric acid to form titanium sulfate and ammonium sulfate, dissolving said sulfates in water, heating the solution thus formed until a titanium hydrate containing a small amount of  $\text{SO}_4$  radical 45 is precipitated, separating the precipitate from the solution, washing the precipitate and treating it with a barium compound to form barium sulfate with the  $\text{SO}_4$  radical present, and calcining the resulting product to form 50  $\text{TiO}_2$  and barium sulfate.
- 55 10. The process of preparing titanium compounds from titaniferous materials containing iron, which comprises heating a titaniferous material containing iron together with carbon in an atmosphere of nitrogen until a titanium nitrogen compound is formed and the iron present is re-

duced to the metallic state, dissolving said metallic iron in dilute sulfuric acid and separating the solution from the residue containing the titanium nitrogen compound, heating said residue together with sulfuric acid to form titanium sulfate and ammonium sulfate, dissolving said sulfates in water, heating the solution thus formed until a titanium hydrate containing a small amount of  $\text{SO}_4$  radical 65 is precipitated, separating the precipitate from the solution, washing the precipitate and treating it with a barium compound to form barium sulfate with the  $\text{SO}_4$  radical present, and calcining the resulting product to form 70 crystalline  $\text{TiO}_2$ .

11. In the recovery of titanium from titaniferous material, the process which comprises the step of heating the titaniferous material in the presence of nitrogen, and a reducing agent, at such temperatures and for such a time that decomposition of the titaniferous material is effected and a titanium nitrogen compound formed. 80

12. In the recovery of titanium from titaniferous material containing iron, the process which comprises the step of heating the titaniferous material in the presence of nitrogen and a reducing agent, at such temperatures and for such a time that decomposition of the titaniferous material is effected, and a titanium nitrogen compound 90 formed and the iron reduced to a metallic state. 95

13. In the recovery of titanium and titaniferous materials containing iron, the process which comprises the step of heating the titaniferous material with carbon in the presence of nitrogen, at such temperature and for such a time that decomposition of the titaniferous material is effected and a titanium nitrogen compound 100 formed and the iron reduced to a metallic state. 105

14. The process of preparing titanium oxygen compounds from titaniferous materials containing iron, which comprises heating the material together with a reducing agent in an atmosphere of nitrogen until a decomposition is effected and a titanium nitrogen compound is formed and the iron reduced to a metallic state, removing the iron from the decomposition product, subjecting the remainder of the 110 said product to further treatment whereby a titanium oxygen compound is formed, and recovering the said compound. 115

Signed at Christiania, Norway, on this 5th day of February, 1918.

PEDER FARUP